

June 28, 1932.

W. R. KAPPES

1,865,192

METHOD OF MAKING STRUCTURAL MATERIAL

Filed March 26, 1931 2 Sheets-Sheet 1

*Fig. 1.*



*Fig. 4.*



*Fig. 2.*



INVENTOR

*W. Raymond Kappes*  
BY *W. Kappes*

ATTORNEY

June 28, 1932.

W. R. KAPPES

1,865,192

METHOD OF MAKING STRUCTURAL MATERIAL

Filed March 26, 1931 2 Sheets-Sheet 2



Fig. 3.

INVENTOR

*W. Raymond Kappes*  
BY *W. G. Smith*

ATTORNEY

## UNITED STATES PATENT OFFICE

WALTER RAYMOND KAPPES, OF OAKMONT, PENNSYLVANIA, ASSIGNOR TO ALUMINUM COMPANY OF AMERICA, OF PITTSBURGH, PENNSYLVANIA, A CORPORATION OF PENNSYLVANIA

## METHOD OF MAKING STRUCTURAL MATERIAL

Application filed March 26, 1931. Serial No. 525,481.

This invention relates to a process for the production of improved insulating material of the type known as "pulp board" or "fiber board".

5 An object of the invention is to produce a fibrous material which is light and porous and has improved heat and sound insulating properties. The term "structural units" as used throughout the specification and 10 claims relates to blocks, boards, sheets or other desirable forms of material suitable for the formation or lining of walls, floors, buildings, containers or other structures where it is desirable that they be resistant 15 to either heat or sound.

A further object of the invention is to produce such porous structural units from materials consisting primarily of pulp or fiber, such as wood pulp, corn stalk, bagasse, jute, 20 flax, hemp or other plant fiber, or other fibrous cellulosic material or asbestos fiber or rock wool or similar inorganic fibrous materials.

I have found that highly porous fibrous 25 structures may be produced by incorporating in a pulp or fiber mass a small amount of a material capable of reacting with a reagent to produce a gas, which gas will exert a leavening effect upon the pulp mass so as to 30 form therein minute bubbles of gas and to produce in the finally shaped and dried mass an extremely light and porous structure suitable particularly for heat or sound insulating purposes.

35 In practicing my invention, I prepare a pulp mass of the nature above described by mixing any suitable fiber stock in a beater or other mixing apparatus with a sufficient amount of water or other solution to render 40 the pulp more or less coherent and sufficiently fluid for satisfactory handling. Such masses as may be thus or similarly formed are referred to herein and in the appended claims as "pulped mass". To the pulp mass 45 thus formed, I add and incorporate uniformly therein a small amount of a leavening agent, i. e., a substance which is capable of producing, by reaction with a suitable reagent, a relatively large amount of gas. 50 This leavening substance may be either a

metal which is capable of reacting with an acid or an alkali, or a chemical compound which is capable of reacting with a suitable reagent to produce the gaseous evolution desired. But in the practice of my invention, 55 I have found it generally preferable to use as the leavening agent a metal in the form of a powder and to act upon the metal powder with an alkali or an acid. Although a chemical compound, such as for instance, 60 calcium carbonate, may be used as a leavening agent to produce the results of my invention, I have found the use of a metal powder to be superior to the use of chemical compounds; for it is desirable from a production stand- 65 point, as will hereinafter be explained, that the start of the leavening action in the pulp mass be delayed slightly from the time that the gas producing agents are added and, furthermore, that the evolution of gas extend 70 over a relatively long interval of time. A metal powder incorporated in the pulp mass is, I have discovered, a material which more readily meets these conditions than a chemical compound in that the metal powders are 75 somewhat slower to react with the acid or alkali which is added to produce the leavening effect and, because of their slowness of action, afford a sufficient opportunity for forming the pulp and obtaining the maxi- 80 mum leavening effect in the pulp mass. Moreover, the reaction between metal powder and acids and alkalies is capable of a more positive regulation of the speed of gas evolution than are mixtures of chemical com- 85 pounds and reagents capable of acting upon them to form a gas.

Among the metal powders which may be used as leavening agents for this purpose are 90 finely divided aluminum, zinc, and magnesium. In the practice of my invention, I have found that in relation to these and other metals, the most satisfactory and commercially practical method of producing a 95 leavening effect in the pulp mass is to add to the mass finely divided or powdered aluminum and to subsequently act upon the aluminum with an alkali, which treatment will produce hydrogen as the leavening gas. 100 Finely divided zinc may be incorporated in

the pulp mass and the gas produced by the addition of either an acid or alkali material, and magnesium will give satisfactory results under the same conditions when treated with an acid. It is preferred, however, to use finely divided aluminum with a subsequent treatment with an alkali for this combination lends itself most readily to the problems of the speed of the gas evolution as outlined above.

10 The amount of leavening agent, whether metal or compound, which should be incorporated in the pulp mass to obtain the best results will vary with the metal or compound to be used and with the amount of leavening action which it is desired to obtain. The necessary amount may be readily predetermined by experiment. Amounts of finely divided aluminum corresponding in weight 15 to about 5 per cent of the dry weight of the fiber stock present in a paper pulp mass have been found to be satisfactory. The amount of leavening action which takes place in the pulp mass is directly a function of the 20 amount of the leavening agent, whether it be metal powder or a chemical compound, incorporated therein and when it is desired to obtain a highly porous, relatively bulky finished product, higher percentages of the 25 leavening agent should be used than when it is desired to produce a product which is not so light and porous and somewhat stiffer and stronger. Generally, the most desirable 30 type of product is obtained by incorporating 35 about 2 to 3 per cent by weight of aluminum powder in the pulp mass.

40 The metal or compound may be incorporated either with the fiber stock before beating or with the liquid pulp mass. I prefer, however, to add the leavening agent to the prepared pulp mass, as a more even distribution throughout the pulp mass is thereby obtained and the leavening action is consequently more uniform and a uniform and 45 satisfactory product is obtained.

50 After the pulp mass containing the leavening agent has been prepared, it is treated with a reagent which will react with the leavening agent to produce the desired leavening action. This reagent is preferably an acid or an alkali which will produce a positive 55 gas producing reaction with the metal or compound used. Where the nature of the pulped material prohibits the use of such reagents, a reagent of another type, such as mercuric chloride, will produce the desired effect. In general, depending upon the 60 nature of the pulped material and the desired speed and volume of gas evolution, any 65 reagent which will produce, with the metal or compound incorporated in the pulped mass, a gas evolution may be satisfactorily used if it is not inherently destructive of the 70 final result desired.

75 The reagent is readily handled in the form

of a solution or suspension in water. When added to the pulp mass in this form, an even distribution throughout the pulp mass may be readily obtained. The amount of reagent to be added may be readily predetermined by 80 calculating the amount required to react with the amount of leavening agent added to the pulped mass. The solution of the reagent should be of such a concentration that too great a bulk of solution is not required to 85 provide a sufficient quantity of the reagent in the pulp mass to substantially completely react with the metal or compound previously incorporated therein. I have found it desirable, however, to use an excess of the reagent over the amount required for complete 90 reaction. But the excess of reagent should not in any case be great since the excess left in the pulp mass after the reaction is completed may have a modifying effect on the 95 fibers in the pulp mass which will substantially change the physical properties of the final product. It is preferred, therefore, to use the reagent in an amount sufficient to give only a slight excess over that required to react with the metal or compound previously incorporated in the pulp mass.

100 When, as in the preferred practice of my invention, finely divided aluminum is added to the pulp mass and the mixture treated with an alkaline reagent to produce a leavening gas, there are certain alkaline reagents to be preferred. I have found that a solution of caustic soda will be satisfactory in those instances where rapid handling of the pulp mass is feasible. Where the rapid handling of the pulp is not feasible, I prefer to use some less active alkaline reagent, and, for this purpose, I have found a suspension of lime in water to be most satisfactory. When such a reagent is used, the evolution of gas is slow in starting and proceeds slowly and regularly, thus affording a reasonable interval for handling and forming the pulp mass before the leavening action has reached its maximum. The maximum advantage of the leavening action is thus secured and a more porous product is obtained. A further advantage accruing from the use of milk of lime arises from the fact that the hydrate of calcium, being only weakly basic, has very little, if any, modifying effect upon the fibrous material. The reagent can, therefore, be used in reasonably large excess if desired without danger of 110 injuring the final product. In fact, it has been found that the product may be materially improved for some purposes by using a relatively large amount of milk of lime in treating the pulp mass. The lime deposited in the fibers from the suspension has a 115 binding quality which renders the finished product stronger and more rigid and also more fire resistant.

120 In the formation of the pulp mass into light, porous structural units, a reasonable

amount of care in handling is required. It is preferred that both the leavening agent and the reagent solution be added to the pulp mass before the forming operation begins so that the pulp mass can be thoroughly agitated in a suitable mixing apparatus. This mix should then be transferred to the forming apparatus without delay as it is preferable that any violent handling of the mass be avoided while the principal part of the leavening action is proceeding. The forming apparatus should be of such a type that the principal part of the water content may be removed from the leavened pulp mass either by drainage or by suction or pressure. In so removing the water, care must be taken, when either suction or pressure is used, that such suction or pressure be very light, otherwise the entrapped gas bubbles may be removed from the leavened mass, causing the whole mass to collapse into a dense and relatively non-porous form.

In practicing my invention, I may employ an apparatus such as illustrated in the accompanying drawings, but it will be understood that this mechanism is shown by way of illustration only, and various other convenient means may be employed to accomplish the results herein described.

30 In the drawings, Fig. 1 represents in perspective view a simple form of apparatus for carrying out my invention;

Fig. 2 represents in perspective view a porous block formed in the apparatus shown in Fig. 1;

Fig. 3 represents in diagrammatic form an arrangement by means of which my invention may be practiced on a commercial scale;

Fig. 4 represents a vertical section on the line 4—4 of Fig. 3.

In Fig. 1, a simple form of apparatus is shown by means of which suitable structural units of pulp mass may be formed. A shallow tray 14 having a perforated bottom 15 of fine screen is positioned above a vacuum hood 16. The pulp mass containing the leavening material may be poured onto the tray and permitted to stand for a short time until the leavening action has become vigorous throughout the mass. The excess liquid is then removed from the pulp mass by applying a slight vacuum beneath the pulp mass and the tray may then be transferred to an oven to completely dry the pulp cake thus formed. By careful handling, the pulp cake may be removed from the shallow tray before drying in the oven if desired.

By means of this apparatus, a stiff block of highly porous, fibrous material as shown in Fig. 2 is produced.

Figs. 3 and 4 represent in diagrammatic form an apparatus in which such structural units may be produced, in accordance with my invention, on a commercial scale.

65 A pulp mass containing a leavening agent,

and in quantity sufficient to fill a form of the desired shape, such as form 6, is run into a rotary mixer 1 through the chute 2. A suitable quantity of reagent is then added to the mixer 1 from the tank 3 by means of the pipe 4, a valve 5 being provided in the pipe line 4 to regulate the quantity of reagent. The pulp mass and the alkali solution are mixed for a suitable period in the rotary mixer 1 and the mixture is then discharged into the form 6, the dot-and-dash line indicating the discharging position of the rotary mixer. The form 6 is provided with a perforated bottom similar to that shown at 2 in Fig. 1. Forms 6 are supported upon a suitable endless conveyor consisting of roller chains 9, and are provided with supporting members 10 which are adapted to ride upon the cross links in the conveyor chains 9 as shown in detail in Fig. 4. Rotatably mounted idler rollers 11 are positioned to support the conveyor chains intermediate the drive sprockets.

A form 6, after having been filled, moves to a second station where, if it is desired to limit the thickness of the block to be formed, a perforated cover 7 of predetermined weight may be placed on the surface of the mixture in the form. The form is then moved to a third station and positioned over the vacuum hood 8 where the liquid is removed from the pulp mass by means of a slight vacuum produced by the vacuum apparatus 12. From this point, the form passes on to the drying oven 13 where the pulp mass is thoroughly dried.

Successive forms are placed on the conveyor and filled and carried intermittently through the successive stations as described, the controlling time interval for movement of the conveyor being the time of mixing and pouring into a form a batch of the pulp mass.

The results which may be obtained in the practice of my invention are illustrated in the following examples. To 300 grams of a pulp mass, there was added 0.5 gram of a milk of lime prepared by adding 100 grams of lime to one liter of water. As soon as the gas was evolved vigorously, a light suction was applied to the mass. This suction was continued until all the excess water had been removed from the pulp. The pulp cake was then transferred to an oven and dried thoroughly. The resulting product was a very light, porous block which was quite firm. The dried block had a weight of 45 grams and an average thickness of 0.5 inch and a bulk of about 25 cubic inches.

To another batch of 300 grams of wet pulp, 1.0 gram of finely divided aluminum powder was added. This mixture was treated with 100 cc. of milk of lime and formed into a dried block as in the preceding experiment. The dried block resulting from this experi-

ment had a weight of 45 grams and a thickness of 0.75 inch and a bulk of about 40 cubic inches.

In a third experiment, 2.0 grams of aluminum powder were added to 300 grams of the wet pulp mass and the mixture was treated with 100 cc. of milk of lime. A dry block was formed of this mass as in the preceding experiments. The resulting product had a weight of 52 grams and a thickness of 1.375 inches.

It will be readily apparent from these examples that the porosity and thickness of the insulating product may be regulated by the amount of metal powder or chemical compound used to produce the leavening gas.

As an example of the results obtained when the amount of lime used is materially increased, a milk of lime containing 200 grams of lime in 600 cc. of water was prepared. This suspension was added to 400 grams of wet pulp mass containing 2 grams of aluminum powder. The resulting mixture was formed and dried as usual. The product obtained was a porous block which was quite strong and rigid. It weighed 275 grams and had a thickness of 1.75 inches.

I claim:

1. The method of making light, porous structural units from pulped masses, comprising mixing with a pulped mass about 2 to 3 per cent of aluminum powder and a predetermined quantity of an alkaline reagent.
2. The method of making light, porous structural units from pulped masses, comprising mixing with a pulped mass a predetermined quantity of metallic powder and a reagent capable of reacting with the metallic powder to produce a leavening gas.
3. The method of making light, porous structural units from pulped masses, comprising mixing with a pulped mass a predetermined quantity of aluminum powder and a predetermined quantity of an alkaline reagent.
4. The method of making light, porous structural units from pulped masses, comprising mixing with a pulped mass a predetermined quantity of aluminum powder, and treating the mixture thus formed with a reagent capable of reacting with said powder to form a leavening gas.
5. A method of making light, porous structural units from pulped masses, comprising adding to the pulped mass a solid leavening agent and a reagent capable of reacting with said leavening agent to form a leavening gas.
6. The method of making light, porous structural units from pulped masses, comprising mixing with a pulped mass a predetermined quantity of metallic powder and an amount of a reagent capable of reacting with said powder to form a leavening gas in ex-

cess of that theoretically required to react with all of said powder.

7. A method of making light, porous structural units from pulped masses, comprising mixing with a pulped mass metallic powder and a reagent capable of reacting with the metallic powder to produce a leavening gas.

8. The method of forming light, porous structural units from pulped masses, comprising forming a pulped mass, incorporating in said mass a solid leavening agent, treating the mixture thus formed with a reagent capable of reacting with said leavening agent to form a leavening gas, and placing the final mixture in a form.

W. RAYMOND KAPPES.

70

75

80

85

90

95

100

105

110

115

120

125

130